



US008551692B1

(12) **United States Patent**  
De Brabander et al.

(10) **Patent No.:** US 8,551,692 B1  
(45) **Date of Patent:** Oct. 8, 2013

(54) **FORMING A FUNNEL-SHAPED NOZZLE**

(75) Inventors: **Gregory De Brabander**, San Jose, CA (US); **Mark Nepomnishi**, San Jose, CA (US); **John A. Higginson**, San Jose, CA (US)

|                  |        |                     |
|------------------|--------|---------------------|
| 2008/0143785 A1  | 6/2008 | Houjou              |
| 2009/0073241 A1* | 3/2009 | Sim et al. ....     |
| 2010/0053270 A1  | 3/2010 | Xu et al.           |
| 2010/0141709 A1  | 6/2010 | De Brabander et al. |
| 2012/0001986 A1* | 1/2012 | Kim .....           |

347/68

347/47

(73) Assignee: **FUJIFILM Corporation**, Tokyo (JP)

(\*) Notice: Subject to any disclaimer, the term of this patent is extended or adjusted under 35 U.S.C. 154(b) by 0 days.

(21) Appl. No.: **13/460,503**

(22) Filed: **Apr. 30, 2012**

(51) **Int. Cl.**  
**B41J 2/16** (2006.01)

(52) **U.S. Cl.**  
USPC ..... 430/320; 430/323; 430/330; 216/27

(58) **Field of Classification Search**

None

See application file for complete search history.

(56) **References Cited**

U.S. PATENT DOCUMENTS

4,857,477 A 8/1989 Kanamori  
5,258,332 A 11/1993 Horioka et al.

JP 2007-175992 A \* 7/2007  
WO 2008/050287 5/2008

FOREIGN PATENT DOCUMENTS

JP 2007-175992 A \* 7/2007

WO 2008/050287 5/2008

OTHER PUBLICATIONS

Computer-generated translation of JP 2007-175992 (Jul. 2007).\*  
Extended European Search Report in EP Application No. 13164670.  
5, dated Aug. 9, 2013, 7 pages.

\* cited by examiner

*Primary Examiner* — John A. McPherson

(74) *Attorney, Agent, or Firm* — Fish & Richardson P.C.

(57) **ABSTRACT**

Techniques are provided for making a funnel-shaped nozzle in a semiconductor substrate. The funnel-shaped recess includes a straight-walled bottom portion and a curved top portion having a curved sidewall gradually converging toward and smoothly joined to the straight-walled bottom portion, and the curved top portion encloses a volume that is substantially greater than a volume enclosed by the straight-walled bottom portion.

13 Claims, 8 Drawing Sheets





FIG. 1



FIG. 2A



FIG. 2B



FIG. 2C



FIG. 3A



FIG. 3B



FIG. 3C



FIG. 4A



FIG. 4B



FIG. 4C



FIG. 4D



FIG. 4E



FIG. 4F



*FIG. 4G*



*FIG. 4H*



FIG. 5A



## 1

## FORMING A FUNNEL-SHAPED NOZZLE

## BACKGROUND

This specification relates to nozzle formation in a micro-electromechanical device, such as an inkjet print head.

Printing a high quality, high resolution image with an inkjet printer generally requires a printer that accurately ejects a desired quantity of ink at a specified location on a printing medium. Typically, a multitude of densely packed ink ejecting devices, each including a nozzle and an associated ink flow path are formed in a print head structure. The ink flow path connects an ink storage unit, such as an ink reservoir or cartridge, to the nozzle. The ink flow path includes a pumping chamber. In the pumping chamber, ink can be pressurized to flow toward a descender region that terminates in the nozzle. The ink is expelled out of an opening at the end of the nozzle and lands on a printing medium. The medium can be moved relative to the fluid ejection device. The ejection of a fluid droplet from a particular nozzle is timed with the movement of the medium to place a fluid droplet at a desired location on the medium.

Various processing techniques can be used to form the ink ejectors in the print head structure. These processing techniques can include layer formation, such as deposition and bonding, and layer modification, such as etching, laser ablation, punching and cutting. The techniques that are used can differ depending on desired nozzle shapes, flow path geometry, along with the materials used in the inkjet printer, for example.

## SUMMARY

A funnel-shaped nozzle having a straight-walled bottom portion and a curved top portion is disclosed. The curved top portion of the funnel-shaped nozzle gradually converges toward and is smoothly joined to the straight-walled bottom portion. The funnel-shaped nozzle can have one or more side surfaces around an axis of symmetry, and cross-sections of the curved top portion and the straight-walled bottom portion in planes perpendicular to the axis of symmetry are geometrically similar. In addition, the curved top portion of the funnel-shaped nozzle encloses a substantially greater volume than the straight-walled bottom portion does, while the straight-walled bottom portion has sufficient height to maintain jetting straightness of fluid droplets ejected through the funnel-shaped nozzle.

To fabricate a funnel-shaped nozzle described in this specification, first, a uniform layer of photoresist is deposited on the planar top surface of a semiconductor substrate. Then, the uniform layer of photoresist is patterned in a regular patterning process (e.g., UV exposure followed by resist development), and an opening created in the uniform layer of photoresist has one or more sidewalls that are substantially perpendicular to the planar top surface of the semiconductor substrate and the planar top surface of the layer of photoresist. Then, the patterned layer of photoresist is heated in vacuum such that the photoresist material in the layer softens and reflows under the influence of gravity and surface tension of the photoresist material. As a result of the reflow, the angled corners on or between the top edge(s) of the opening become rounded and the top edge(s) transform into a single rounded edge. The radius of curvature of the rounded edge can be controlled by the reflow bake conditions. For example, the radius of curvature of the rounded edge can be equal or greater than the initial thickness of the uniform layer of photoresist deposited on the semiconductor substrate. After the desired

## 2

rounded shape of the top edges is obtained, the patterned layer of photoresist is allowed to cool and re-harden, while the rounded shape of the top edges remains.

After formation of the patterned layer of photoresist that has the opening with a curved side surface gradually expanding toward and smoothly joined to an exposed top surface of the patterned layer of photoresist, the forming of a funnel-shaped recess in the semiconductor substrate can begin.

First, a straight-walled recess is etched in the semiconductor substrate through the patterned layer of photoresist, for example, using a Bosch process. The high-selectivity etching of the straight-walled recess leaves the layer of photoresist substantially un-etched. The depth of the recess can be a few microns less than the final designed height of the funnel-shaped nozzle. The horizontal cross-sectional shape of the funnel-shaped recess can be circular, oval, or polygonal, and is determined by the lateral shape of the opening in the patterned layer of photoresist. Once the straight-walled recess is formed in the semiconductor substrate, a dry etching process is started to transform the straight-walled recess into the funnel-shaped recess. Specifically, the etchant used in the dry etching have comparable (e.g., substantially equal) etch rates for both the photoresist and the material of the semiconductor substrate (e.g., a Si <100> wafer). During the dry etching, the etchant gradually deepens the straight-walled recess to form a straight-walled bottom portion of the funnel-shaped recess. At the same time, the dry etching expands the vertical sidewall(s) of the straight-walled recess into a curved side surface that levels off into the horizontal top surface of the semiconductor substrate at the top, and converges toward and smoothly transitions into the straight-walled bottom portion of the funnel-shaped recess. The curved side surface created during the dry etching forms the curved top portion of the funnel-shaped recess and encloses a volume substantially greater than the volume enclosed by the straight-walled bottom portion. The funnel-shaped recess can be opened at the bottom either by continued etching or by removing the unetched substrate from below.

In one aspect, a process for making a nozzle for ejecting fluid droplets includes forming a patterned layer of photoresist on a top surface of a semiconductor substrate, the patterned layer of photoresist including an opening, the opening having a curved side surface smoothly joined to an exposed top surface of the patterned layer of photoresist. The top surface of the semiconductor substrate is etched through the opening in the patterned layer of photoresist to form a straight-walled recess, the straight-walled recess having a side surface substantially perpendicular to the top surface of the semiconductor substrate; and After the straight-walled recess is formed, the patterned layer of photoresist and the semiconductor substrate are dry etched, where the dry etching gradually thins the patterned layer of photoresist along a surface profile of the patterned layer of photoresist while transforming the straight-walled recess into a funnel-shaped recess. The funnel-shaped recess includes a straight-walled bottom portion and a curved top portion having a curved sidewall gradually converging toward and smoothly joined to the straight-walled bottom portion, and the curved top portion encloses a volume that is substantially greater than a volume enclosed by the straight-walled bottom portion.

Implementations can include one or more of the following features Forming the patterned layer of photoresist on the top surface of the semiconductor substrate may include depositing a uniform layer of photoresist on the top surface of the semiconductor substrate, creating an initial opening in the uniform layer of photoresist, where the initial opening has a side surface substantially perpendicular to an exposed top

surface of the uniform layer of photoresist, after the initial opening is created in the uniform layer of photoresist, softening the uniform layer of photoresist by heat until a top edge of the initial opening becomes rounded under the influence of surface tension, and after the softening by heat, re-hardening the uniform layer of photoresist while the top edge of the initial opening remains rounded. The uniform layer of photoresist may be deposited on the top surface of the semiconductor substrate is at least 10 microns in thickness. Softening the uniform layer of photoresist by heat may include heating the uniform layer of photoresist having the initial opening formed therein in a vacuum environment until photoresist material in the uniform layer of photoresist reflows under the influence of surface tension. Heating the uniform layer of photoresist may include heating the uniform layer of photoresist to a temperature of 160-250 degrees Celsius. Re-hardening the uniform layer of photoresist may include cooling the uniform layer of photoresist in a vacuum environment while the top edge of the initial opening remains rounded. A top opening of the curved top portion may be at least four times as wide as a bottom opening of the curved top portion. Etching the top surface of the semiconductor substrate to form the straight-walled recess may include etching the top surface of the semiconductor substrate through the opening in the patterned layer of photoresist using a Bosch process. The dry etching to form the funnel-shaped recess may have substantially the same etch rates for the patterned layer of photoresist and the semiconductor substrate. The dry etching to form the funnel-shaped recess may form at least part of the curved top portion underneath the patterned layer of photoresist. The dry etching to form the funnel-shaped recess may include dry etching using a  $\text{CF}_4/\text{CHF}_3$  gas mixture. The opening in the patterned layer of photoresist may have a circular cross-sectional shape in a plane parallel to the exposed top surface of the patterned layer of photoresist. The funnel-shaped recess may have a circular cross-sectional shape in a plane parallel to the top surface of the semiconductor substrate.

In another aspect, an apparatus for ejecting fluid droplets includes a semiconductor substrate having a funnel-shaped nozzle formed therein. The funnel-shaped nozzle includes a straight-walled bottom portion and a curved top portion having a curved side surface gradually converging toward and smoothly joined to the straight-walled bottom portion. The funnel-shaped recess has an axis of symmetry substantially perpendicular to a top surface of the semiconductor substrate. A volume enclosed by the curved top portion is substantially greater than a volume enclosed by the straight-walled bottom portion.

Implementations may include one or more of the following features. A top opening of the curved top portion may be at least 70 microns wider than a bottom opening of the curved top portion within a plane containing the axis of symmetry. The straight-walled bottom portion may have a width of 30-40 microns in a plane including the axis of symmetry. The straight-walled bottom portion may have a height of 5-10 microns in a plane containing the axis of symmetry. A straight line coplanar with the axis of symmetry and intersecting a top opening and a bottom opening of the curved top portion may be at an angle of 30-40 degrees from the axis of symmetry. The straight-walled bottom portion may have a height that is 10-30% of a width of the straight-walled bottom portion in a plane containing the axis of symmetry. The funnel-shaped nozzle may be one of an array of identical funnel-shaped nozzles, and each of the array of identical funnel-shaped nozzle belongs to an independently controllable fluid ejection unit. A piezoelectric actuator assembly may be supported on

a top surface of the semiconductor substrate and including a flexible membrane sealing a pumping chamber fluidly connected to the funnel-shaped nozzle. Each actuation of the flexible membrane may be operable to eject a fluid droplet through the straight-walled bottom portion of the funnel-shaped nozzle. A volume enclosed by the curved top portion may be three or four times a size of the fluid droplet.

Particular implementations can include none, one or more of the following advantages.

The funnel-shaped nozzle has a curved top portion whose volume is sufficiently large to hold several droplets (e.g., 3 or 4 droplets) of fluid. The side surface of the funnel-shaped nozzle is streamlined and free of discontinuities in the fluid ejection direction. Compared to a straight-walled nozzle (e.g., a cylindrical nozzle) of the same depth and drop size, the side surface of the funnel-shaped nozzle generates less friction on the fluid during fluid ejection, and prevents the nozzle from taking in air when the droplet breaks free from the nozzle. Reducing the fluid friction not only improves the stability and uniformity in droplet formation, but also allows faster jetting frequencies, lower driving voltages, and/or higher power efficiencies. Preventing air from entering the nozzle can help prevent trapped air bubbles from blocking the nozzle or other parts of the flow path.

Although a nozzle having tapered, flat sidewalls (e.g., a nozzle of an inverted pyramid shape) may also realize some advantages (e.g., reduced friction) over a cylindrical nozzle, the sharp angled edges at the bottom opening of tapered nozzle still pose more drag on the droplets than the funnel-shaped nozzle does. In addition, the angled edges and rectangular (or square) shape of the tapered nozzle opening also affect the straightness of the drop direction in an unpredictable way, leading to deterioration of printing quality. In the funnel-shaped nozzle described in this specification, the straight-walled bottom portion accounts for only a small portion of the overall nozzle depth, thus, the straight-walled bottom portion ensures jetting straightness without causing too much friction on fluid being expelled. Thus, the funnel-shaped nozzle can help achieve better jetting straightness, higher firing frequencies, higher power efficiencies, lower driving voltages, and/or uniformity of drop shape and locations.

Although funnel-shaped nozzles having a curved side surface may be formed using electroforming or micro-molding techniques, such techniques are limited to metal or plastic materials and may not be workable in forming nozzles in semiconductor substrates. In addition, the electroforming or micro-molding techniques tend to have lower precision and cannot achieve the size, geometry, and pitch requirements needed for high-resolution printing. The semiconductor processing techniques can be used to produce large arrays of nozzles that are highly compact and uniform, and can meet the size, geometry, and pitch requirements needed for high-resolution printing. For example, nozzles can be as small as 5 microns, the nozzle-to-nozzle pitch accuracy can be about 0.5 microns or less (e.g. 0.25 microns), the first nozzle-to-last nozzle pitch accuracy can be about 1 micron, and the nozzle size accuracy can be at least 0.6 microns.

The details of one or more embodiments of the invention are set forth in the accompanying drawings and the description below. Other features, objects, and advantages of the invention will be apparent from the description and drawings, and from the claims.

#### DESCRIPTION OF DRAWINGS

FIG. 1 shows a cross-sectional side view of an apparatus for fluid droplet ejection.

FIG. 2A is a cross-sectional side view of a print head flow path with a nozzle having a single straight sidewall (i.e., a cylindrical nozzle), and a top plan view of the nozzle.

FIG. 2B is a cross-sectional side view of a print head flow path with a nozzle having tapered, flat sidewalls, and a top plan view of the nozzle.

FIG. 2C is a cross-sectional side view of a print head flow path with a nozzle having a tapered top portion abruptly joined to a straight-walled bottom portion, and a top plan view of the nozzle.

FIG. 3A is a cross-sectional side view of a funnel-shaped nozzle having a curved top portion smoothly joined to a straight-walled bottom portion.

FIG. 3B is a top plan view of a funnel-shaped nozzle having a curved top portion smoothly joined to a straight-walled bottom portion, where the horizontal cross-sectional shapes of the nozzle are circular.

FIG. 3C is a cross-sectional side view of a print head flow path with a nozzle having a tapered top portion smoothly joined to a straight-walled bottom portion.

FIGS. 4A-4H illustrate the process for making a funnel-shaped nozzle having a curved top portion smoothly joined to a straight-walled bottom portion.

FIGS. 5A and 5B shows images of two funnel-shaped recesses made using the process shown in FIGS. 4A-4G.

Like reference symbols in the various drawings indicate like elements.

#### DETAILED DESCRIPTION

Fluid drop ejection can be implemented with a substrate, for example, a microelectromechanical system (MEMS), including a fluid flow body, a membrane, and a nozzle layer. The flow path body has a fluid flow path formed therein, which can include a fluid filled passage, a fluid pumping chamber, a descender, and a nozzle having an outlet. An actuator can be located on a surface of the membrane opposite the flow path body and proximate to the fluid pumping chamber. When the actuator is actuated, the actuator imparts a pressure pulse to the fluid pumping chamber to cause ejection of a droplet of fluid through the outlet of the nozzle. Frequently, the flow path body includes multiple fluid flow paths and nozzles, such as a densely packed array of identical nozzles with their respective associated flow paths. A fluid droplet ejection system can include the substrate and a source of fluid for the substrate. A fluid reservoir can be fluidically connected to the substrate for supplying fluid for ejection. The fluid can be, for example, a chemical compound, a biological substance, or ink.

Referring to FIG. 1, a cross-sectional schematic diagram of a portion of a microelectromechanical device, such as a printhead in one implementation is shown. The printhead includes a substrate 100. The substrate 100 includes a fluid path body 102, a nozzle layer 104, and a membrane 106. The nozzle layer 104 is made of a semiconductor material, such as silicon. A fluid reservoir supplies a fluid to a fluid fill passage 108. The fluid fill passage 108 is fluidically connected to an ascender 110. The ascender 110 is fluidically connected to a fluid pumping chamber 112. The fluid pumping chamber 112 is in close proximity to an actuator 114. The actuator 114 can include a piezoelectric material, such as lead zirconium titanate (PZT), sandwiched between a drive electrode and a ground electrode. An electrical voltage can be applied between the drive electrode and the ground electrode of the actuator 114 to apply a voltage to the actuator and thereby actuate the actuator. A membrane 106 is between the actuator

114 and the fluid pumping chamber 112. An adhesive layer (not shown) can secure the actuator 114 to the membrane 106.

A nozzle layer 104 is secured to a bottom surface of the fluid path body 102 and can have a thickness between about 5 15 and 100 microns. A nozzle 117 having an outlet 118 is formed in an outer surface 120 of the nozzle layer 104. The fluid pumping chamber 112 is fluidically connected to a descender 116, which is fluidically connected to the nozzle 117.

10 While FIG. 1 shows various passages, such as a fluid fill passage, pumping chamber, and descender, these components may not all be in a common plane. In some implementations, two or more of the fluid path body, the nozzle layer, and the membrane may be formed as a unitary body. In 15 addition, the relative dimensions of the components may vary, and the dimensions of some components have been exaggerated in FIG. 1 for illustrative purposes.

The design of the flow path, the nozzle dimensions and shape in particular, affect printing quality, printing resolution, as well, energy efficiencies of the printing device. FIGS. 2A-2C show a number of conventional nozzle shapes.

For example, FIG. 2A shows a print head flow path 202 with a straight nozzle 204. The straight nozzle 204 has a straight sidewall 206. The top portion of FIG. 2A shows a cross-sectional side view of the flow path 202 and the nozzle 204 in a plane passing through a central axis 208 of the nozzle 204. The central axis 208 is an axis that passes through the geometric center of all the horizontal cross-sections of the nozzle 204. In this specification, the central axis 208 of the nozzle is sometimes referred to as the axis of symmetry of the nozzle in cases where the geometric center of each horizontal cross section is also the center of symmetry of the horizontal cross section. As indicated in the top portion of FIG. 2A, in a plane including the central axis 208, the profile of the sidewall 206 are straight lines parallel to the central axis 208. In this example, the nozzle 204 is a circular right cylinder, and has a single straight sidewall. In other examples, the nozzle can be a square right cylinder, and has four straight, flat side surfaces.

40 As shown in FIG. 2A, the nozzle 204 is formed in a nozzle layer 210. The nozzle 204 has the same cross-sectional shapes and sizes in planes perpendicular to the central axis 208 of the nozzle 204. The lower portion of FIG. 2A shows the top plan view of the nozzle layer 210. In this example, the nozzle 204 45 has a circular cross-sectional shape in the planes perpendicular to the central axis 208 of the nozzle 204. In various implementations, the nozzle 204 can have other cross-sectional shapes, such as oval, square, rectangular, or other regular polygonal shapes.

50 A nozzle having straight sidewall(s) is relatively easy to fabricate. The straight sidewall(s) of the nozzle can help maintain jetting straightness and making the landing positions of ink droplets ejected from the nozzle more predictable. However, to ensure a sufficient drop size, the height of the 55 straight-walled nozzle needs to be rather large (e.g., tens of microns or more). The large vertical dimension of the straight-walled nozzle creates a significant amount of friction on the fluid inside the nozzle, when the fluid is ejected from the nozzle as a droplet. The higher flow resistance created in the straight-walled nozzle results in a lower jetting frequency, and/or a higher driving voltage, which can further lead to lower printing speed, lower resolution, lower power efficiency, and/or lower device life.

Another drawback of the straight-walled nozzle is that, 60 when a droplet breaks free from the outlet (e.g., outlet 212) of the nozzle, air can be sucked into the nozzle from the outlet opening of the nozzle and be trapped inside the nozzle or

other parts of the flow path. The air trapped inside the nozzle can block ink flow or deflect fluid droplets that are being ejected from their desired trajectory.

FIG. 2B shows a print head flow path 214 with a nozzle 216 having tapered, flat sidewalls 218. The upper portion of FIG. 2B shows a cross-sectional side view of the print head flow path 214 in a plane containing the central axis 220 of the nozzle 216. In the plane containing the central axis 220, the profile of the nozzle 216 are straight lines converging toward the central axis 220 going from the top opening of the nozzle 216 to the bottom opening (or outlet 212) of the nozzle 216. The profile of the nozzle 216 can be formed by multiple planes that converge toward the center axis 220.

The nozzle 216 is formed in a nozzle layer 224, and the cross-sectional shapes of the nozzle 216 in planes perpendicular to the central axis 220 are squares of continuously decreasing sizes. The nozzle 216 have four flat sidewalls each slanted from an edge of the top opening of the nozzle 216 to a corresponding edge of the bottom opening of the nozzle 216. The lower portion of FIG. 2B shows a top plan view of the nozzle layer 224. As shown in the lower portion of FIG. 2B, each sidewall 218 of the nozzle 216 is a flat surface that intersects with each of two adjacent flat sidewalls 218 along an edge 226. Each edge 226 is an angled edge, rather than a rounded edge.

As shown in the lower portion of FIG. 2B, the lower opening of the nozzle 216 is a smaller square opening while the upper opening of the nozzle 216 is a larger square opening. The central axis 220 passes through the geometric centers of both the upper opening and the lower opening of the nozzle 216. The tapered sidewalls 218 of the nozzle 216 provides reduced friction on the fluid passing through the nozzle as compared to the straight-walled nozzle 204 shown in FIG. 2A. The tapered shape of the nozzle 216 also reduces the amount of air intake occurring during the breakup of droplets at the nozzle outlet 212.

The tapered nozzle 216 shown in FIG. 2B can be formed in a semiconductor nozzle layer 224 (e.g., a silicon nozzle layer) using KOH etching. However, the shape of the tapered nozzle 216 is dictated by the crystal planes existing in the semiconductor nozzle layer 224. When the nozzle 216 is created by KOH etching, the side surfaces of the nozzle 216 are formed along the <111> crystal planes of the semiconductor nozzle layer 224. Therefore, the angle between each slanted side surface 218 and the central axis 220 has a fixed value of about 35 degrees.

Although the tapered nozzle 216 shown in FIG. 2B offers some improvement over the straight-walled nozzle 204 shown in FIG. 2A in terms of lowered flow resistance and reduced air uptake, there is very little flexibility in terms of changing the shape of the nozzle opening or the angle of the tapered sidewalls. The square corners of the nozzle outlet can sometimes cause satellites (tiny secondary droplets created in addition to a main droplet during droplet ejection) to form. In addition, the sharp discontinuities between the flat sidewalls 218 and the horizontal bottom surface of the nozzle layer 224 at the edges of the nozzle outlet 212 also cause additional drag on the droplets, causing reduced jetting speed and frequency.

FIG. 2C shows another nozzle configuration that combines a tapered section as shown in FIG. 2B with a straight section as shown in FIG. 2A. Due to the limitation posed by the KOH etching techniques, the straight bottom portion and the tapered top portion are formed by etching from two sides of the substrate. However, the two-side etching can lead to difficult alignment issues. Otherwise, specially designed steps have to be taken to form the straight bottom portion from the

same side as the tapered portion, e.g., as described in U.S. Patent Publication 2011-0181664, incorporated by reference.

The top portion of FIG. 2C shows a cross-sectional side view of a print head flow path 232 with a nozzle 234 having a tapered top portion 236 abruptly joined to a straight bottom portion 238. The cross-sectional side view shown in FIG. 2C is in a plane containing the central axis 240 of the nozzle 234. In the plane containing the central axis 240, the profile of the tapered top portion 236 consists of straight lines converging from the top opening of the nozzle 234 toward the intersection between the tapered top portion 236 and the straight-walled bottom portion 238. In the plane containing the central axis 240, the profile of the straight-walled bottom portion 238 consists of straight lines parallel to the central axis 240. This profile can be provided by a cylinder that is co-axial with the central axis 240. The intersection between the tapered top portion 236 and the straight-walled bottom portion 238 is not smooth and has one or more discontinuities or angled edges in the vertical direction (i.e., the fluid ejection direction in this example).

In this example, the cross-sectional shapes of the tapered top portion 236 in planes perpendicular to the central axis of the nozzle 234 are square, while the cross-sectional shapes of the bottom portion 238 in planes perpendicular to the central axis of the nozzle 234 are circular. Therefore, the tapered top portion 236 has four flat side surfaces 244 each slanted from an edge of the top opening of the tapered top portion 236 to a corresponding edge of the intersection between the top portion 236 and the bottom portion 238. Although the straight bottom portion 238 shown in FIG. 2C has a circular cross-section, the straight bottom portion can also have a square cross-section or cross-sections of other shapes.

The nozzle 234 is formed in the nozzle layer 242. The lower portion of FIG. 2C shows the top plan view of the nozzle 234. In the top plan view, the lower opening of the straight-walled bottom portion 238 is circular, and the top opening of the tapered top portion 236 is square, and the intersection between the straight bottom portion 238 and the tapered top portion 236 is an intersection between a cylindrical hole and an inverted pyramid hole. Due to the mismatch between the cross-sectional shapes between the top and bottom portions, the edges of the intersection include curves and sharp discontinuities. These discontinuities also cause fluid friction and instability in drop formation. Even if the cross-sectional shapes of the top portion 236 and the bottom portion 238 are both square, there are still discontinuities at the intersection between the two portions in the fluid ejection direction. The square-shaped nozzle opening is also less ideal than a circular nozzle outlet for other reasons set forth with respect to FIG. 2B, for example.

In this specification, a funnel-shaped nozzle having a curved top portion smoothly joined to a straight-walled bottom portion formed in a semiconductor nozzle layer (e.g. silicon nozzle layer) is disclosed. The curved top portion of the funnel-shaped nozzle differs from a tapered top portion shown in FIG. 2C in that the profile of the side surface of the curved top portion in a plane containing the central axis of the nozzle consists of curved rather than straight lines. In addition, the profile of the curved top portion converges toward the straight bottom portion and is smoothly joined to the straight-walled bottom portion, rather than bending at an abrupt angle at the intersection between the curved top portion and the straight-walled bottom portion.

In addition, in some implementations, the transition from the horizontal top surface of the nozzle layer to the curved side surface of the funnel-shaped nozzle is also smooth rather than abrupt. In addition, the horizontal cross-sectional shapes

of the funnel-shaped nozzle in planes perpendicular to the central axis of the nozzle are geometrically similar and concentric for the entire depth of the nozzle. Therefore, there is no jagged intersection between the curved top portion and the straight-walled bottom portion of the funnel-shaped nozzle. The funnel-shaped nozzle described in this specification offer many advantages over the conventional nozzle shapes described with respect to FIGS. 2A-2C, for example.

FIG. 3A is a cross-sectional side view of a funnel-shaped nozzle 302 having a curved top portion 304 smoothly joined to a straight-walled bottom portion 306. In the straight walled bottom portion 306, the sides of the nozzle are parallel, and are perpendicular to the outer surface 322 of the nozzle layer. The straight-walled bottom portion 306 can be a cylindrical passage (i.e., the walls are straight up/down rather than laterally). The funnel-shaped nozzle 302 is a funnel-shaped through hole formed in a planar semiconductor nozzle layer 308. The intersection between the curved top portion 304 and the straight-walled bottom portion 306, whose location is indicated by the dotted line 320 in FIG. 3A, is smooth and substantially free of any discontinuities and any surfaces perpendicular to the central axis 310 of the nozzle 302.

As shown in FIG. 3A, the height of the curved top portion 304 is substantially larger than the height of the straight-walled bottom portion 306. However, the straight-walled bottom portion 306 has at least some height, e.g., 10-30% of the height of the curved top portion 304. For example, the height of the curved top portion 304 can be 40-75 microns (e.g., 40, 45, or 50 microns), while the height of the bottom portion 306 can be only 5-10 microns (e.g., 5, 7, or 10 microns). The curved top portion 304 encloses a volume much larger than the straight-walled bottom portion 306. The larger curved top portion holds most of the fluid to be ejected. In some implementations, the volume enclosed in the curved top portion 304 is the size of several droplets (e.g., 3 or 4 droplets). Each droplet can be 3-100 picoliters. The straight bottom portion 306 has a smaller volume, such as a volume less than the size of a single droplet.

The height of the straight-walled portion 306 is small enough so that it does not cause a significant amount of fluid friction, and does not cause substantial air uptake during break-off of the droplets. At the same time, the height of the straight-walled portion is large enough to maintain jetting straightness. In some implementations, the height of the straight-walled portion 306 is about 10-30% of the diameter of the nozzle outlet. For example, in FIG. 3A, the nozzle outlet has a diameter of 35 microns, and the height of the straight-walled portion is 5-10 microns (e.g., 7 microns). In some implementations, the diameter of the nozzle outlet can be 15-45 microns.

Both the curved top portion 304 and the straight-walled bottom portion 306 of the nozzle 302 serve important functions in droplet formation and ejection. The curved top portion 304 is designed to hold a sufficient volume of fluid so that when a droplet is ejected from the nozzle outlet, there is little or no void created in the nozzle to form air bubbles inside the nozzle. At the same time, the straight-walled bottom portion holds a much smaller volume of fluid, and serves to maintain jetting straightness without causing any significant drag on the fluid droplet during jetting.

The funnel-shaped nozzle 302 further differs from the nozzles shown in FIGS. 2B and 2C in that the cross-sectional shape of the funnel-shaped nozzle 302 in planes perpendicular to the central axis 310 of the nozzle 302 are circular, rather than rectangular, for the entire depth of the nozzle 302. Thus, there is no discontinuity between the curved top portion 304 and the straight bottom portion 306 in the direction of fluid

ejection. The streamlined profile of the funnel-shaped nozzle 302 provides even less fluid friction than the nozzles shown in FIGS. 2B and 2C. In addition, the side surface of the funnel-shaped nozzle 304 is completely smooth and free of any discontinuities or abrupt changes in the azimuthal direction as well. Therefore, the funnel-shaped nozzle 304 does not produce drag or instabilities to cause other drawbacks (e.g., satellite formation) present in the nozzles shown in FIG. 2B and FIG. 2C either.

It can be difficult to form a funnel-shape nozzle in silicon using conventional etching processes. Conventional etching processes, such as the Bosch process, form straight vertical walls, whereas and KOH etching which forms tapered, straight walls. Although isotropic etching can form curved features, like bowl-shaped features, it is not able to make curved walls in the opposite formation to make funnel-shaped features.

In addition, given the processing techniques provided in this specification, the pitch by which the curved top portion of the funnel-shaped nozzle converges from its top opening towards the straight-walled bottom portion can be varied by design, rather than fixed by the orientation of certain crystal planes. Specifically, suppose that point A is the intersection between the edge of the top opening of the curved top portion 304 and a plane containing the central axis 310, and point B is the intersection between the edge of the bottom opening of the curved top portion 304 and the same plane containing the central axis 310. Unlike the nozzle 234 shown in FIG. 2C, the angle  $\alpha$  between a straight line joining the point A and point B and the central axis 310 is not a fixed angle (e.g., 35 degrees in FIG. 2C) dictated by the crystal planes of the semiconductor nozzle layer 308. Instead, the angle  $\alpha$  for the funnel-shaped nozzle 304 can be designed by varying the processing parameters when making the funnel-shaped nozzle 304. In some implementations, the angle  $\alpha$  for the funnel-shaped nozzle 304 can be between 30-40 degrees. In some implementations, the angle  $\alpha$  for the funnel-shaped nozzle 304 can be greater than 40 degrees.

As is shown in FIG. 3A, the curved top portion 304 of the funnel-shaped nozzle 302 differ from a rounded lip resulted from a natural rounding or tapering of a recess wall created in the process of creating a cylindrical recess in a substrate.

First, the amount of tapering exhibited by the curved top portion 304 of the funnel-shaped recess 302 is much larger than any tapering that might be inherently present due to manufacturing imprecisions (e.g., over etching of substrate through a straight-walled photoresist mask). For example, the angle of tapering for the sidewall of a funnel-shaped nozzle is about 30 to 40 degrees. The vertical extent of the curved top portion 304 can be tens of microns (e.g., 50-75 microns). The width of the top opening of the curved top portion 304 can be 100 microns or more, and can be 3 or 4 times the width of the bottom opening of the curved top portion 304. In contrast, the tapering or rounding present near the top opening of a cylindrical recess due to manufacturing imperfections and/or imprecisions is typically less than 1 degree. The natural tapering or rounding also has a much smaller height and width variation (e.g., in the range of nanometers or less than 1-2 microns) than those present in the funnel-shaped nozzle 302 described in this specification.

FIG. 3B is a top plan view of a funnel-shaped nozzle (e.g., the nozzle 302 shown in FIG. 3A). As shown in FIG. 3B, the top opening 312 and the bottom opening 314 of the funnel-shaped nozzle 302 are both circular and are concentric. There is no discontinuity at any part of the side surface 316 of the entire nozzle 302. The width of the top opening 312 is at least 3 times the width of the bottom opening 314 of the nozzle 302.

## 11

In some implementations, the top opening 312 of the nozzle 302 is fluidically connected to a pumping chamber above the funnel-shaped nozzle 302, and the boundary of the pumping chamber defines the boundary of the top opening 312 of the funnel-shaped nozzle 302. FIG. 3C shows a print head flow path 318 with a funnel-shaped nozzle 302.

Although FIG. 3B shows a funnel-shaped nozzle having a circular cross-sectional shape for its entire depth, other cross-sectional shapes are possible. The cross-sectional shape of the straight-walled bottom portion of a funnel-shaped nozzle can be oval, square, rectangular, or other polygonal shapes. The curved top portion of the funnel-shaped nozzle would have a similar cross-sectional shape as the straight-walled bottom portion. However, the corners (if any) in the cross-sectional shape of the curved top portion are gradually eliminated or smoothed out as the side surface of the curved top portion extends further away from the straight-walled bottom portion toward the top opening of the curved top portion. The exact shape of the cross-sections of the curved top portion is determined by the manufacturing steps and the materials used for creating the funnel-shaped nozzles.

For example, in some implementations, the funnel-shaped nozzle having a curved top portion smoothly joined to a straight-walled bottom portion can have a square horizontal cross-sectional shape. In such implementations, the center side profile of the nozzle is the same as that shown in FIG. 3A. However, the funnel-shaped nozzle would have four converging curved side surfaces, and the intersections between adjacent curved side surfaces are four smooth curved lines converging toward the bottom outlet of the nozzle and smoothly transition into four straight parallel lines in the straight bottom portion of the nozzle. In addition, the intersections between adjacent curved side surfaces are smoothly rounded, so that the four curved side surfaces form part of a single smooth side surface in the top portion of the funnel-shaped nozzle.

A print head body can be manufactured by forming features in individual layers of semiconductor material and attaching the layers together to form the body. The flow path features that lead to the nozzles, such as the pumping chamber and ink inlet, can be etched into a substrate, as described in U.S. patent application Ser. No. 10/189,947, filed Jul. 3, 2002, using conventional semiconductor processing techniques. A nozzle layer and the flow path module together form the print head body through which ink flows and from which ink is ejected. The shape of the nozzle through which the ink flows can affect the resistance to ink flow. By creating a funnel-shaped nozzle described in this application, less flow resistance, higher jetting frequencies, lower driving voltages, and/or better jetting straightness can be achieved. The processing techniques described in this specification also allow arrays of nozzles having the desired dimensions and pitches to be made with good uniformity and efficiencies.

FIGS. 4A-4H illustrate the process for making a funnel-shaped nozzle having a curved top portion smoothly joined to a straight-walled bottom portion, for example, the funnel-shaped nozzle shown in FIGS. 3A-3C.

To form the funnel-shaped nozzle, first, a patterned layer of photoresist is formed on a top surface of a semiconductor substrate, where the patterned layer of photoresist includes an opening that has a curved side surface smoothly joined to an exposed top surface of the patterned layer of photoresist. For example, an opening around a z-axis will have a side surface that curves in both the z direction and the azimuthal direction. The shape of the opening will determine the cross-sectional shapes of the funnel-shaped nozzle in planes perpendicular to the central axis of the funnel-shaped nozzle. The size of the

## 12

opening is roughly the same as the bottom opening of the funnel-shaped nozzle (e.g., 35 microns). In the example shown in FIGS. 4A-4H, the opening is circular for making a funnel-shaped nozzle having circular horizontal cross-sections throughout the entire depth of the nozzle.

To form the patterned layer of photoresist, a resist-reflow process can be used. As shown in FIG. 4A, a uniform layer of photoresist 402 is applied to the planar top surface 404 of a semiconductor substrate 406 (e.g., a silicon wafer). The semiconductor substrate 406 can be a substrate having one of several crystal orientations, such as a silicon <100> wafer, a silicon <110> wafer, or a silicon <111> wafer. The thickness of the layer of photoresist 402 influences the final curvature of the curved side surface of the opening in the layer of photoresist, and hence the final curvature of the curved side surface of the funnel-shaped nozzle. A thicker layer of photoresist is generally applied to obtain a larger radius of curvature for the curved side surface of the funnel-shaped nozzle.

In this example, the initial thickness of the uniform layer of photoresist 406 is about 10-11 microns (e.g., 11 microns). In some implementations, more than 11 microns of photoresist can be applied on the planar top surface 404 of the semiconductor substrate 406. Some thickness of photoresist can remain on the substrate after the processing steps to make the funnel-shaped recess of a desired depth. Examples of the photoresist that can be used include AZ 9260, AZ9245, AZ4620 made by MicroChemicals® GmbH, and other positive photoresists, for example. The thickness of the semiconductor substrate 406 is equal or greater than the desired depth for the funnel-shaped nozzle to be made. For example, the substrate 406 can be an SOI wafer having a silicon layer of about 50 microns attached to a handle layer via a thin oxide layer. Alternatively, the substrate 406 can be a thin silicon layer attached to a handle layer by an adhesive layer or by Van der Waals force.

As shown in FIG. 4B, after the uniform layer of photoresist 402 is applied to the planar top surface 404 of the semiconductor substrate 406, the uniform layer of photoresist 402 is patterned, such that an initial opening 408 having one or more vertical side walls 410 are created. In this example, a circular opening is created in the uniform layer of photoresist 402, and the sidewall of the circular opening is a single curved surface that is perpendicular to the planar top surface 412 of the uniform layer of photoresist 402 and to the planar top surface 404 of the semiconductor substrate 406. The diameter of the initial circular opening 408 determines the diameter of the bottom opening of the funnel-shaped nozzle to be made. In this example, the diameter of the initial circular opening 408 can be about 20-40 microns (e.g., 35 microns). The patterning of the uniform layer of photoresist 402 can include the standard UV or light exposure under a photomask and a photoresist development process to remove the portions of the photoresist layer exposed to the light.

After the initial opening 408 is formed in the uniform layer of photoresist 402, the photoresist layer 402 is heated to about 160 to 250 degrees Celsius and until the photoresist material in the layer 402 is softened. When the photoresist material in the patterned layer of photoresist 402 is softened under the heat treatment, the photoresist material will start to reflow and reshape itself under the influence of surface tension of the photoresist material, particularly in regions near the top edge 414 of the opening 408. The surface tension of the photoresist material causes the surface profile of the opening 408 to pull back and become rounded. As shown in FIG. 4C, the top edge 414 of the opening 408 have become rounded under the influence of surface tension.

In some implementations, the layer of photoresist 402 is heated in a vacuum environment to achieve the reflow of the photoresist layer 402. By heating the photoresist layer 402 in a vacuum environment, the surface of the photoresist layer 402 is more smooth and without tiny air bubbles trapped inside of the photoresist material. This will lead to better surface smoothness in the final nozzle produced. The amount by which the top edge 414 of the circular opening 408 is pulled back and rounded is influenced by the lateral size of the circular opening 408, the thickness of the photoresist layer 402, as well as the weight and viscosity of the photoresist material. These parameters can be adjusted to achieve the desired amount of expansion achieved in the top edge 414 of the opening 408 once the reflow occurs.

After the desired shape of the opening 408 is obtained, the photoresist layer 402 is cooled. The cooling can be accomplished by removing the heat source or active cooling. The cooling can also be performed in a vacuum environment to ensure better surface properties of the funnel-shaped nozzle to be made. By cooling the photoresist layer 402, the photoresist layer 402 re-harden, and the surface profile of the opening 408 maintains its shape during the hardening process, and the top edge 414 of the opening 408 remain rounded at the end of the re-hardening process, as shown in FIG. 4D.

Once the patterned layer of photoresist 402 is hardened, the etching of the substrate 406 can begin. The funnel-shaped recess is created in a two-step etching process. First, a straight-walled recess is created in a first etching process. Then, the straight-walled recess is modified during a second etching process. In the second etching process, the initially formed straight-walled recess is deepened to form the straight-walled bottom portion of the funnel-shaped recess. At the same time, the second etching process expands the initially formed straight-walled recess gradually from the top to form the curved top portion of the funnel-shaped recess.

As shown in FIG. 4E, an initial straight-walled recess 416 is created through the patterned layer of photoresist 402 in a first etching process. The first etching process can be a Bosch process, for example. In the first etching process, a straight walled recess 416 is created and has a depth slightly smaller (e.g., 5-15 microns less) than the final desired depth of the funnel-shaped recess to be made. For example, for a funnel-shaped recess having a total depth of 50-80 microns, the straight-walled recess 416 created in the first etching process can be 45-75 microns. Although tiny scalloping patterning may be present on the side profile 418 of the straight-walled recess 416, such small variations (e.g., 1 or 2 degrees) is small compared to the overall dimensions (e.g., 35 microns in width and 45-75 microns in depth) of the straight-walled recess 416.

In the first etching process, the straight-walled recess 416 has substantially the same cross-sectional shape and size in a plane parallel to the top surface 404 of the semiconductor substrate 406 as the area enclosed by the bottom edge of the opening 408 in the photoresist layer 402. As shown in FIG. 4E, the etchant used in the first etching process removes very little of the photoresist layer 402 as compared to the semiconductor substrate 406 exposed through the opening 408 in the photoresist layer. Therefore, the surface profile of the patterned layer of photoresist 402 remains substantially unchanged at the end of the first etching process. For example, the selectivity between the semiconductor substrate 406 and the photoresist layer 402 during the first etching process can be 100:1.

After the initial straight-walled recess 416 is formed in the semiconductor substrate 406 through the first etching process, the second etching process can be started to transform

the initial straight-walled recess 416 shown in FIG. 4E into the desired funnel-shaped recess 420 shown in FIG. 4F.

As shown in FIG. 4F, the semiconductor substrate 406 and the patterned layer of photoresist 402 are exposed to dry etching from the vertical direction (e.g., the direction perpendicular to the planar top surface 404 of the substrate 406 in FIG. 4F). The etchant used in the dry etching process can have comparable etch rates for both the photoresist and for the semiconductor substrate 406. For example, the selectivity of the dry etching between the photoresist and the semiconductor substrate can be 1:1. In some implementations, the dry etching is performed using a  $\text{CF}_4/\text{CHF}_3$  and  $\text{O}_2$  gas mixture at high platen power, e.g., greater than 400 W.

During the dry etching, as the etching process continues, the surface profile of the photoresist layer 402 recedes in the vertical direction under the bombardment of the etchant. Due to the curved profile 414 at the top edge of the opening 408 in the photoresist layer 402, the surface of the semiconductor substrate 406 under the thinnest portion of the photoresist layer 402 gets exposed to the etchant first, as compared to other parts of the substrate surface underneath of the photoresist layer 402. The portions of the semiconductor surface exposed to the etchant also are gradually etched away. As shown in FIG. 4F, the dotted lines represent the surface profiles 414 of the photoresist layer 402 and the semiconductor substrate 406 receding gradually under the bombardment of the etchant.

As the dry etching continues, some undercutting beneath the photoresist layer 402 can occur. For example, as shown in FIG. 4F, the regions 422 below the edge of the opening 408 in the photoresist layer 402 are etched, and the surface of the semiconductor substrate 406 are expanded in the lateral direction. The expanded side surface 418 of the recess 416 becomes the curved side surface 424 of the curved top portion of the funnel-shaped recess 420 formed in the semiconductor substrate 406.

As the dry etching continues to expand the side surface 418 of the recess 416 in the lateral direction, the dry etching also deepens the recess 416 in the vertical direction. The deepening of the recess 416 creates the straight-walled bottom portion of the funnel-shaped recess 420. The additional amount of deepening creates a straight-walled portion that is a few microns deep. The side surface 426 of the straight-walled bottom portion is perpendicular to the planar top surface 404 of the semiconductor substrate 406. Since the amount of lateral expansion of the side surface 424 of the recess 420 gradually decreases from top to bottom, the curved side surface 424 of the curved top portion transitions smoothly into the vertical side surface 426 of the straight-walled bottom portion. The boundary of the top opening of the funnel-shaped recess 420 is defined by the edge starting from which the photoresist meets the surface of the substrate 406.

The dry etching can be timed and stopped as soon as the desired depth of the funnel-shaped recess 420 is reached. Alternatively, the dry etching is timed and stopped as soon as the desired surface profile for the curved portion of the funnel-shaped recess 420 is obtained.

In some implementations, if the semiconductor substrate is of the desired thickness of the nozzle layer, the dry etching can be continued until the etching goes through the entire thickness of the semiconductor substrate, and the funnel-shaped nozzle is formed completely. In some implementations, the semiconductor substrate can be etched, ground and/or polished from the backside until the funnel-shaped recess is opening from the backside to form the funnel-shaped nozzle.

## 15

The photoresist 402 is removed, and FIG. 4G shows a completed funnel-shaped recess 428 that has been opened at the bottom. After the funnel-shaped nozzle 428 is formed, the nozzle layer 406 can be attached to other layers of a fluid ejection unit, such as a fluid ejection unit 430 shown in FIG. 4H. In some implementations, the funnel-shaped nozzle 428 is one of an array of identical funnel-shaped nozzles, and each of the arrays of identical funnel-shaped nozzle belongs to an independently controllable fluid ejection unit 430. In some implementations, a fluid ejection unit includes a piezoelectric actuator assembly supported on the top surface of the semiconductor substrate 406 and including a flexible membrane sealing a pumping chamber fluidly connected to the funnel-shaped nozzle 428. Each actuation of the flexible membrane is operable to eject a fluid droplet through the straight-walled bottom portion of the funnel-shaped nozzle 428, and a volume enclosed by the curved top portion is three or four times a size of the fluid droplet.

FIGS. 5A and 5B shows images of two funnel-shaped recesses (e.g., recess 502 and recess 504) made using the process shown in FIGS. 4A-4G.

The dimensions of the funnel-shaped recess may be different in different implementations. As shown in FIG. 5A, the straight-walled bottom portion 506 of the funnel-shaped recess 502 has a depth of about 30 microns, while the curved top portion 508 of the funnel-shaped recess 502 has a depth of about 37 microns. When creating a funnel-shaped nozzle out of this funnel-shaped recess 502, the substrate can be ground and polished from the bottom, such that the straight-walled portion 506 has the desired depth, such as 5-10 microns. As shown in FIG. 5A, the diameter of the straight-walled bottom portion 506 is roughly uniform (with a variation of less than ~0.5 microns for a 20 micron diameter) in planes perpendicular to the central axis of the recess 502. The bottom opening of the curved top portion 508 is smoothly joined to the top opening of the straight-walled bottom portion 506. The diameter of the top opening of the recess 502 is in the range of 126 microns, 6 times the diameter of the straight-walled bottom portion 506. The pitch by which the curved top portion 508 expands from the bottom to the top can be defined by the width of the curved top portion 508 at half height of the curved top portion 508. In this example, the width at half height of the curved top portion is about 34 microns.

In FIG. 5B, a shallower funnel-shaped recess 504 is formed. The top opening of the curved top portion 510 has a diameter of about 75 microns, and is about 4.4 times the diameter of the straight-walled bottom portion 512. The total height of the funnel-shaped recess 504 is about 49 microns, and the height of the straight-walled bottom portion 512 is about 4 microns. The width at half height of the curved top portion 510 is about 30 microns.

A number of implementations of the invention have been described. Nevertheless, it will be understood that various modifications may be made without departing from the spirit and scope of the invention. Exemplary methods of forming the aforementioned structures have been described. However, other processes can be substituted for those that are described to achieve the same or similar results. Accordingly, other embodiments are within the scope of the following claims.

What is claimed is:

1. A process for making a nozzle for ejecting fluid droplets, the process comprising:

forming a patterned layer of photoresist on a top surface of a semiconductor substrate, the patterned layer of photoresist including an opening, the opening having a curved side surface smoothly joined to an exposed top surface of the patterned layer of photoresist;

## 16

etching the top surface of the semiconductor substrate through the opening in the patterned layer of photoresist to form a straight-walled recess, the straight-walled recess having a side surface substantially perpendicular to the top surface of the semiconductor substrate; and after the straight-walled recess is formed, dry etching the patterned layer of photoresist and the semiconductor substrate, where the dry etching gradually thins the patterned layer of photoresist along a surface profile of the patterned layer of photoresist while transforming the straight-walled recess into a funnel-shaped recess, the funnel-shaped recess includes a straight-walled bottom portion and a curved top portion having a curved sidewall gradually converging toward and smoothly joined to the straight-walled bottom portion, and the curved top portion encloses a volume that is substantially greater than a volume enclosed by the straight-walled bottom portion.

2. The process of claim 1, wherein forming the patterned layer of photoresist on the top surface of the semiconductor substrate comprises:

depositing a uniform layer of photoresist on the top surface of the semiconductor substrate; creating an initial opening in the uniform layer of photoresist, where the initial opening has a side surface substantially perpendicular to an exposed top surface of the uniform layer of photoresist;

after the initial opening is created in the uniform layer of photoresist, softening the uniform layer of photoresist by heat until a top edge of the initial opening becomes rounded under the influence of surface tension; and after the softening by heat, re-hardening the uniform layer of photoresist while the top edge of the initial opening remains rounded.

3. The process of claim 2, wherein the uniform layer of photoresist deposited on the top surface of the semiconductor substrate is at least 10 microns in thickness.

4. The process of claim 2, wherein softening the uniform layer of photoresist by heat further comprises:

heating the uniform layer of photoresist having the initial opening formed therein in a vacuum environment until photoresist material in the uniform layer of photoresist reflows under the influence of surface tension.

5. The process of claim 2, wherein heating the uniform layer of photoresist comprises:

heating the uniform layer of photoresist to a temperature of 160-250 degrees Celsius.

6. The process of claim 2, wherein re-hardening the uniform layer of photoresist comprises:

cooling the uniform layer of photoresist in a vacuum environment while the top edge of the initial opening remains rounded.

7. The process of claim 1, wherein a top opening of the curved top portion is at least four times as wide as a bottom opening of the curved top portion.

8. The process of claim 1, wherein etching the top surface of the semiconductor substrate to form the straight-walled recess comprises:

etching the top surface of the semiconductor substrate through the opening in the patterned layer of photoresist using a Bosch process.

9. The process of claim 1, wherein the dry etching to form the funnel-shaped recess has substantially the same etch rates for the patterned layer of photoresist and the semiconductor substrate.

**10.** The process of claim 1, wherein the dry etching to form the funnel-shaped recess forms at least part of the curved top portion underneath the patterned layer of photoresist.

**11.** The process of claim 1, wherein the dry etching to form the funnel-shaped recess comprises dry etching using a CF<sub>4</sub>/ 5 CHF<sub>3</sub> gas mixture.

**12.** The process of claim 1, wherein the opening in the patterned layer of photoresist has a circular cross-sectional shape in a plane parallel to the exposed top surface of the patterned layer of photoresist. 10

**13.** The process of claim 1, wherein the funnel-shaped recess has a circular cross-sectional shape in a plane parallel to the top surface of the semiconductor substrate.

\* \* \* \* \*